

## 1

3,414,128  
**NITROGENOUS MATERIAL FRACTIONS  
OBTAINED FROM GILSONITE IN FROTH  
FLOTATION**

Robert E. Baarson, La Grange, and Charles L. Ray,  
Wheaton, Ill., assignors, by mesne assignments, to  
Armour Industrial Chemical Company, a corporation  
of Delaware  
No Drawing. Filed Sept. 24, 1965, Ser. No. 490,114  
6 Claims. (Cl. 209—167)

### ABSTRACT OF THE DISCLOSURE

A recovery of molybdenum or molybdenum and copper from metallic sulfide ores is brought about in a flotation operation in which finely-divided metallic sulfide ores containing molybdenum and iron or molybdenum, copper and iron are conditioned with a mixture of heterocyclic nitrogen compounds extracted from the mineral gilsonite and having an average boiling point within the range of about 200° F. to 750° F., the molybdenum or molybdenum and copper being separated as froth product.

This invention relates to nitrogenous material fractions obtained from gilsonite in froth flotation, and more particularly to the use of such material as a collector or auxiliary collector for molybdenum and copper concentrates from metallic sulfide ores.

An object of the invention is to provide new collectors and combinations of collectors for the treatment of metallic sulfide ores containing molybdenum minerals and ores containing copper, molybdenum and iron minerals, and like ores. A further object is to provide a process for utilizing, in the collection of molybdenum and copper concentrates from metallic sulfide ores, nitrogenous material obtained from gilsonite used either alone or in combination with other collectors. A still further object is to provide for the use of synergistic combinations of such nitrogenous material with other collectors for the collection of molybdenum and copper concentrates and for the separation of said concentrates. Other specific objects and advantages will appear as the specification proceeds.

In one embodiment of our invention, nitrogenous material fractions obtained from gilsonite are employed to condition a molybdenum-bearing sulfide pulp together with a frother, if desired, such as methyl amyl alcohol or propylene glycol ether, and following the conditioning, flotation is conducted in the usual manner to effect concentration and recovery of the molybdenum concentrate. We have discovered that such nitrogenous material is particularly effective as a collector for molybdenum concentrates from metallic sulfide ores.

In the foregoing specific embodiment, metallic sulfide ore containing predominantly molybdenum is ground to a finely-divided state and a water pulp of the finely-divided ore is mixed or conditioned with about 0.03 lb. of the collector and about 0.03 lb. of a frother per ton of dry ore. Following conditioning, flotation is conducted

## 2

for several minutes. An additional amount of collector and frother may then be added and flotation continued for another period. The flotation concentrate thus obtained may then be subjected to further upgrading operations in order to produce a concentrate of higher grade. The quantities of collector required may range from about 0.005 lb. to about 0.5 lb. per ton of dry ore, but such range of quantities may vary beyond the above range, depending upon the nature of the ore treated.

Where the metallic sulfide ore contains substantial amounts of copper in addition to molybdenum, we prefer to employ with the nitrogenous material fractions obtained from gilsonite a cooperating collector for simultaneous recovery of copper and molybdenum concentrates, and such concentrates may be separated by depressing the copper concentrate through the use of heat or depressant materials such as Nokes reagent, sodium hydroxide, potassium permanganate, sodium sulfide, sodium ferrocyanide, etc.

The nitrogenous material is derived from mineral gilsonite through distillation, acid extraction, and well known extraction techniques. Such crude mixed heterocyclic nitrogenous material occurs as a by-product in the manufacture of petroleum products from the gilsonite mineral by the American Gilsonite Company. The extreme complexity of the mixture of different compounds in the crude material renders a complete qualitative analysis substantially prohibitive.

The American Gilsonite Company has assigned descriptive nomenclature to various fractions of this type material as follows:

(1) Light Bases from HBF.—Extracted from a naphtha stream of approximately 283° F. volumetric average boiling point and 222° F. to 400° F. boiling range.

(2) Intermediate Bases From PFB.—Extracted from a heavy naphtha stream of approximately 422° F. volumetric boiling point and 400° to 590° F. boiling range.

(3) Medium Bases from LGO.—Extracted from a gas-oil stream of about 520° F. volumetric average boiling point and 460° to 665° F. boiling range.

(4) Semi-purified Acid Extracted Nitrogen Compounds:

(a) Nitrogen Bases I.—Boiling range 491° F. to 509° F. at 760 mm.

(b) Nitrogen Bases II.—Boiling range 610° F. to 641° F. at 760 mm.

(c) Nitrogen Compounds III.—Boiling range 700° to 710° F. at 760 mm.

(d) Nitrogen Compounds IV.—Boiling range 745° to 755° F. at 760 mm.

(e) Bottoms V.—Boiling range 755° F. and higher at 760 mm.

(5) Nitrogen Distillate.—A crude mixture of nitrogen bases obtained by distillation and representative of 4(a) through 4(c) inclusive as above, plus some non-nitrogenous compounds.

(6) Nitrogen Bases Concentrate Oil.—An extracted mixture of cyclic tertiary amines plus some non-basic nitrogen compounds.

(7) Pyrrole Polymer Oil.—An extracted mixture con-

taining predominantly non-basic nitrogen compounds and some cyclic basic nitrogen compounds.

In the practice of the present invention, all of the foregoing fractions which have a boiling range of about 200° to about 700° F., and preferably those having an average boiling point within the range of about 450° to 750° F., may be employed. Best results, however, have been obtained through the use of fraction 6 in the above descriptive outline, namely, nitrogen bases concentrate oil, and fraction 5, nitrogen distillate. By the use of nitrogen bases concentrate oil, which is referred to in the trade and herein as "NBC oil" or "Gilsamine," we have obtained excellent results in recovering molybdenum concentrate from metallic sulfide ores in which molybdenum is the principal metal to be recovered. Similarly, excellent results have been obtained by the use of nitrogen distillate (fraction 5). Where the metallic sulfide ores contain copper as well as molybdenum, we find that the NBC oil and nitrogen distillate are highly effective as auxiliary collectors in the recovery of both molybdenum fractions and copper concentrates. By the term "nitrogenous material obtained from gilsonite," we intend to include fractions 1 to 7, inclusive, in the above-mentioned nomenclature of the American Gilsonite Company, and by the term "nitrogen bases concentrate oil," or "NBC oil," we intend to include fraction 6 as described in such nomenclature. As stated above, the term "nitrogen bases concentrate oil" or "NBC oil" is a term commonly used in the industry and is understood as defining a specific material. Also, the term "nitrogen distillate" is commonly used in the industry and is understood to designate fraction 5 as described in the above descriptive nomenclature.

While NBC oil is regarded in the trade generally as a waste material, we have found it particularly useful and effective as a collector when used alone in the conditioning of metallic sulfide ores containing predominantly molybdenum. Where the ore contains substantial amounts of copper which must be recovered, we prefer to employ the NBC oil together with known collectors such as sodium and potassium xanthate having 2 to 12 carbon atoms, isopropyl ethyl thionocarbamate, alkyl or aryl dithiophosphate, etc. In the case of a copper-bearing mineral in which there is very little molybdenum, the use of the NBC oil aids in the recovery of copper when used in conjunction with the commonly used collectors for copper. Further, it materially aids in the depression of iron pyrite and prevents excessive recovery of this mineral.

We have also discovered that the use of NBC oil with S-substituted isothiouronium salts provides an unusually effective combination of collectors for the recovery of molybdenum and copper concentrates from metallic sulfide ores containing these minerals along with iron minerals. S-substituted isothiouronium salts are preferably prepared by refluxing an alcoholic solution of thiourea with a fatty halide or with an aromatic halide and are represented by the following formula:



where R is an aliphatic (straight chain or branched chain), cycloaliphatic, or aromatic hydrocarbon group having 2 or more but not more than 24 carbon atoms and preferably not more than 8 carbon atoms, or mixtures thereof, and where X is a halide such as Cl, Br, I, etc. Best results have been obtained when the hydrocarbon group has from 4 to 10 carbon atoms. Other methods of preparation of the collectors may be employed.

Specific examples of the collectors may be designated as benzyl-, ethyl-, isopropyl-, n-butyl-, n-amyl-, isoamyl-, 2-ethylhexyl-, n-octyl-, 1-methyloctyl-, dodecyl-, lauryl-, tetradecyl-, and tallow isothiouronium chloride, and other salts as defined above where the fatty halide or aromatic

halide has from 2 to 24 or, preferably, from 2 to 18 carbon atoms and including mixtures of said halides. The preferred collectors have from 4 to 10 carbon atoms in the collector molecules and include n-butyl isothiouronium chloride, n-amyl isothiouronium chloride, and 2-ethylhexyl isothiouronium chloride.

Since the collectors are either water-soluble or water dispersible, it is preferred to apply them to flotation as water solutions or water dispersions ranging from about 1% to about 10% active by weight.

10 Unusually good results have been obtained when the S-substituted isothiouronium salts are employed with NBC oil and also with a known class of collectors which are referred to as "sulphydryl" collectors, which include the alkyl or aryl dithiophosphates, dithiocarbonates (xanthates), dithiocarbamates, thionocarbamates, thioureas, xanthogen formates, and the like, commonly used for flotation treatment of metallic sulfide ores.

15 As specific examples, NBC oil has been employed effectively with n-butyl isothiouronium chloride and with n-amyl isothiouronium chloride and 2-ethylhexyl isothiouronium chloride. Where considerable copper is involved, we prefer to add to each of the combinations above isopropyl ethyl thionocarbamate or sodium or potassium xanthate having from 2 to 12 carbon atoms. Another effective combination has been NBC oil together with alkyl dithiophosphate and isopropyl ethyl thionocarbamate.

20 The proportions of NBC oil to the other collector or collectors may be varied substantially, but for the recovery of copper alone, we prefer to use the proportions of 1:2 to 2:1. A 1:1 ratio has been found very satisfactory. Where both copper and molybdenum are to be recovered, a satisfactory proportion of the NBC oil to the other collector or collectors is 1:2 to 2:1, the preferred proportion being 2:3.

25 After the collection of molybdenum and copper concentrates, any of the commonly-used agents may be employed for the copper-depressing step. For example, Nokes reagent (a reaction product of a material such as sodium hydroxide with a material such as phosphorus pentasulfide) may be used. A combination of heat and an excess of either lime or sodium hydroxide may be employed. Sodium sulfide, or sodium ferrocyanide, or various combinations of the foregoing agents may be employed. We have found that ferrocyanide is particularly useful as a copper-depressing agent when the collectors described above are employed.

30 The invention may be further illustrated by the following examples, which are illustrative of preferred embodiments of the invention, but the invention is not limited thereby.

#### EXAMPLE I

35 A South American ore analyzing 2.8% copper and 0.72% molybdenum was crushed and ground in a laboratory rod mill to pass 96% through -48 mesh. The -48 mesh + 200 mesh fraction was 60% by weight of the total product; the remainder -200 mesh. The product was ground at 50% solids and a 0.01 #/T addition of a collector was added to the mill. Some of the tests were conducted at a pH of 11.5 using lime, and other tests as indicated were conducted at a natural pH 7.5.

40 The ground pulp was diluted to 20% solids in a 500-gram Denver flotation cell, conditioned for 10 sec. with Dowfroth 250, and floated for 2 minutes. After the preliminary flotation, additional flotation steps preceded by small collector additions and conditioning in the cell were made until froths were barren of sulfide minerals. The concentrates were filtered, dried and assayed. The tests were conducted on several different ore samples as indicated in the following Table I.

TABLE I

| Reagent and Test No.                                                    | #/T   | pH    | Rougher Conc. |            | Rougher Tail |            | Rougher Recovery |            |
|-------------------------------------------------------------------------|-------|-------|---------------|------------|--------------|------------|------------------|------------|
|                                                                         |       |       | Percent Cu    | Percent Mo | Percent Cu   | Percent Mo | Percent Cu       | Percent Mo |
| <b>South American Ore #1—2.8% Cu; 0.72% Mo:</b>                         |       |       |               |            |              |            |                  |            |
| Nitrogen Distillate (#485-117)                                          | 0.115 | 7.5   | 19.62         | 5.21       | 0.174        | 0.0444     | 94.8             | 94.4       |
| Nitrogen Distillate (#485-335)                                          | 0.138 | 7.7   | 18.18         | 4.49       | 0.166        | 0.0499     | 95.0             | 93.9       |
| Nitrogen Distillate (#485-118)                                          | 0.115 | 11.2  | 13.85         | 7.26       | 1.65         | 0.0428     | 45.1             | 94.3       |
| Z-200                                                                   | 0.110 | 7.8   | 16.33         | 3.92       | 0.096        | 0.060      | 97.2             | 93.0       |
| Z-11 (Avg. 3 tests) on Ore #485                                         | 0.040 |       |               |            |              |            |                  |            |
| Standard:                                                               |       |       |               |            |              |            |                  |            |
| Z-200                                                                   | 0.06  |       |               |            |              |            |                  |            |
| Z-11 (#485-300)                                                         | 0.02  | 11.55 | 22.76         | 3.69       | 0.097        | 0.290      | 97.0             | 64.1       |
| <b>South American Ore #2, Ore Analysis—1.20% Cu; 1.16% Mo; 8.9% Fe:</b> |       |       |               |            |              |            |                  |            |
| Nitrogen Distillate (#502-16)                                           | 0.168 | 11.2  | 3.17          | 8.73       | 0.87         | 0.098      | 32.4             | 92.2       |
| NBC Oil (#502-17)                                                       | 0.168 | 11.2  | 4.26          | 6.54       | 0.68         | 0.103      | 56.9             | 93.0       |
| Nitrogen Distillate (#502-3)                                            | 0.150 | 7.3   | 3.56          | 10.25      | 0.93         | 0.094      | 29.4             | 92.2       |
| NBC Oil (#502-11)                                                       | 0.150 | 7.3   | 4.41          | 6.24       | 0.58         | 0.161      | 60.0             | 88.5       |
| Z-200                                                                   | 0.06  |       |               |            |              |            |                  |            |
| Z-11 (#502-92)                                                          | 0.02  | 11.5  | 4.15          | 3.34       | 0.151        | 0.492      | 90.2             | 68.7       |
| Z-200                                                                   | 0.03  |       |               |            |              |            |                  |            |
| N-butylisothiouronium Chloride (#502-36)                                | 0.04  | 11.6  | 4.20          | 4.27       | 0.127        | 0.150      | 92.4             | 91.4       |
| <b>Canadian Molybdenum Ore—0.097% Mo; 2.13% Fe:</b>                     |       |       |               |            |              |            |                  |            |
| NBC Oil (22)                                                            | 0.075 | 7.4   | -----         | 9.70       | -----        | 0.025      | -----            | 91.8       |
| Mineral Seal Oil (39)                                                   | 0.06  | 8.1   | -----         | 8.44       | -----        | 0.024      | -----            | 91.2       |

In the above, nitrogen distillate is used alone as a collector in the treatment of a copper and molybdenum-bearing sulfide ore. Table results show that nitrogen distillate alone is as effective as a normal collector of molybdenum sulfide. Nitrogen distillate tests were conducted at two

## EXAMPLE II

The ore used in both parts of Table II was prepared in the same manner as that outlined in the procedure for Table I. Analyses of the samples are given separately under Table II results.

TABLE II

| Reagent and Test No.                                             | #/T    | pH | Rougher Conc. |            | Rougher Tails |            | Rougher Recovery |            |
|------------------------------------------------------------------|--------|----|---------------|------------|---------------|------------|------------------|------------|
|                                                                  |        |    | Percent Cu    | Percent Mo | Percent Cu    | Percent Mo | Percent Cu       | Percent Mo |
| <b>South American Ore #1 (Same as Ex. #1) 2.80% Cu, 0.72 Mo:</b> |        |    |               |            |               |            |                  |            |
| Nitrogen Distillate                                              | 0.092  |    |               |            |               |            |                  |            |
| Z-200                                                            | 0.05   |    |               |            |               |            |                  |            |
| Z-11 (#485-328)                                                  | 0.0167 |    |               |            |               |            |                  |            |
| Z-200                                                            | 0.06   |    |               |            |               |            |                  |            |
| Z-11                                                             | 0.02   |    |               |            |               |            |                  |            |
| <b>South American Ore #2—1.20% Cu, 1.16% Mo, 8.97% Fe:</b>       |        |    |               |            |               |            |                  |            |
| NBC Oil                                                          | 0.07   |    |               |            |               |            |                  |            |
| Z-11 (#502-39)                                                   | 0.06   |    |               |            |               |            |                  |            |
| Z-200                                                            | 0.06   |    |               |            |               |            |                  |            |
| Z-11                                                             | 0.02   |    |               |            |               |            |                  |            |

different pH's and as far as bulk flotation was concerned at the neutral pH of 7.5-7.7 the nitrogen distillate floated both the sulfide and molybdenum minerals almost completely. At a pH of 11.2 (the commonly used pH in commercial operations), the copper minerals were depressed and a higher recovery of molybdenum minerals was obtained which is a desirable trend where separation of the two minerals may be required later in steps. It will also be noted that with a standard collector system, Z-11 and Z-200 at the operating pH of 11.0-11.5, the molybdenum is not floated as effectively as with the nitrogen distillate.

The second part of the example records the comparison of nitrogen distillate and NBC oil as collectors. The nitrogen distillate was an early fraction considered semi-commercial and later replaced by NBC oil. NBC oil not only replaces the nitrogen distillate, but is favored.

The third part of the example records the effectiveness of NBC oil at a neutral operating pH against a standard oil used in the field on a straight molybdenum ore.

The last two examples emphasize the effectiveness of NBC oil alone as regards recovery on ores containing predominately molybdenum sulfide and little copper sulfide minerals, or straight molybdenum ores.

Nitrogen distillate and NBC oil are believed to be replacements for each other and either can be used.

The purpose of this example was to observe the effectiveness of nitrogen distillate and NBC oil and commonly used sulphydryl collectors on two different ores. It will be noted that in every case where nitrogen distillate and NBC oil was used the sulphydryl collectors against the standard collectors there is a considerable improvement in the molybdenum recovery and noted improvement in copper sulfide recovery at this normal pH for commercial operations. This shows synergism; in fact, the recovery of molybdenum is very markedly improved with the addition of nitrogen distillate or NBC oil to sulphydryl-type collectors.

## Example III

Two different ore samples were treated in the example shown in Table III. The ore designated as Ore No. 3 was an ore from southwestern United States, with an analysis of 0.81% copper and 0.012% molybdenum sulfide. The ore was crushed to pass through a 65 mesh screen retaining 40% on the +200 mesh screen. The ore samples were ground at 50% solids with 0.025 #/T of the collector selected and with sufficient lime to give a pulp pH of 10.5. This was followed by a 5-minute flotation time and 20-second conditioning time, with cresylic acid used as a frother.

TABLE III

| Reagent                                                      | #/T   | pH | Rougher Conc. |            | Rougher Tails |            | Rougher Recovery |            |
|--------------------------------------------------------------|-------|----|---------------|------------|---------------|------------|------------------|------------|
|                                                              |       |    | Percent Cu    | Percent Mo | Percent Cu    | Percent Mo | Percent Cu       | Percent Mo |
| Southwestern U.S. Ore #3—0.81% Cu, 0.012% MoS <sub>2</sub> : |       |    |               |            |               |            |                  |            |
| NBC Oil                                                      | 0.7   |    | 11.5          | 8.0        | 0.086         | 0.153      | 0.0018           | 82.3       |
| n-Amylithiouronium chloride                                  | 0.025 |    |               |            |               |            |                  |            |
| NBC Oil                                                      | 0.07  |    | 11.6          | 8.7        | 0.0655        | 0.170      | 0.0024           | 79.7       |
| n-Butylithiouronium chloride                                 | 0.025 |    |               |            |               |            |                  |            |
| Sodium Aeroflate (Standard Reagent)                          | 0.09  |    | 10.6          | 14.8       | 0.088         | 0.23       | 0.0043           | 73.9       |
| South American Ore #2—1.20% Cu, 1.16% Mo, 8.97% Fe:          |       |    |               |            |               |            |                  |            |
| NBC Oil                                                      | 0.056 |    | 11.6          | 3.95       | 3.91          | 0.128      | 0.1009           | 92.3       |
| n-Amylithiouronium chloride (#502-124)                       | 0.06  |    |               |            |               |            |                  |            |
| NBC Oil                                                      | 0.056 |    | 11.5          | 3.81       | 3.87          | 0.112      | 0.0778           | 93.4       |
| 2-ethylhexyl isothiouronium chloride (#502-122)              | 0.06  |    |               |            |               |            |                  |            |
| Standard:                                                    |       |    |               |            |               |            |                  |            |
| Z-200                                                        | 0.06  |    | 11.5          | 4.15       | 3.34          | 0.151      | 0.402            | 90.2       |
| Z-11                                                         | 0.02  |    |               |            |               |            |                  |            |

The ore designated as Ore No. 2 is the same as that defined in Example I.

tests. The purpose of the testing was to determine the effect of depression of iron sulfide.

TABLE V

| Reagent and Test No. | #/T    | pH | Rougher Conc. |            | Rougher Tail |            | Percent Recovery of Cu and Fe in Concentrate |            |
|----------------------|--------|----|---------------|------------|--------------|------------|----------------------------------------------|------------|
|                      |        |    | Percent Cu    | Percent Fe | Percent Cu   | Percent Fe | Percent Cu                                   | Percent Fe |
| Z-11                 | 0.0165 |    | 10.8          | 6.58       | 29.03        | 0.198      | 0.876                                        | 89.74      |
| Z-200 (#488-31)      | 0.0330 |    |               |            |              |            |                                              |            |
| Z-11 and Nitrogen    | 0.03   |    | 10.2          | 7.10       | 19.80        | 0.178      | 3.37                                         | 90.24      |
| Distillate (#488-19) | 0.03   |    |               |            |              |            |                                              | 57.51      |

This example shows the effective combinations of NBC oil with the isothiouronium salts indicated against the standard reagents on two different ores against two different current standard anionic collectors. In every case there is improvement in recovery of both copper and molybdenum when using the combination over that in using the standard collectors. The improvement in recovery of molybdenum minerals is especially noted.

In comparing the results of NBC oil and Z-11 combination of Table II with the NBC oil-isothiouronium chloride salts of the second part of Table III, the improvement of using isothiouronium chloride with NBC oil can be noted over using current collectors with NBC oil.

#### EXAMPLE IV

Samples of an ore feed of 1.63% Cu and 0.028% Mo were taken from the prepared feed to a South American flotation plant and subjected to laboratory flotation tests.

The effect of depression of iron and improvement in copper recovery is noted.

#### EXAMPLE VI

35 A laboratory flotation test was made of a South American metallic sulfide ore containing molybdenum and copper and iron (2.8% Cu, 0.72% Mo), using on the same ore a number of different collectors in a series of seven tests. The term "nitrogen distillate" indicates a gilsonite distillate corresponding to group 5 in the American Gilsonite Company nomenclature. The xanthate is sodium isopropyl xanthate (Z-11). The thionocarbamate is isopropyl ethyl thionocarbamate (Z-200).

40 In accordance with the test procedure, the grind was at 50% solids and the amount of collector added to the mill varied with the collectors tested. The bulk flotation pH level varied between 7.6 and 11.6. The ground pulps were diluted to about 20% solids in a 1,000-gram stainless steel Denver flotation cell (1800 r.p.m.), conditioned for

TABLE IV

| Test No. | Reagent                                           | #/T   | pH   | Rougher Conc. |            | Rougher Tails |            | Rougher Recovery |            |
|----------|---------------------------------------------------|-------|------|---------------|------------|---------------|------------|------------------|------------|
|          |                                                   |       |      | Percent Cu    | Percent Mo | Percent Cu    | Percent Mo | Percent Cu       | Percent Mo |
| 1        | N-butylithiouronium chloride                      | 0.02  | 11.5 | 27.5          | 0.20       | 0.16          | 0.010      | 90.5             | 47.3       |
| 2        | {N-butylithiouronium chloride<br>HBC Oil}         | 0.015 | 11.5 | 29.6          | 0.21       | 0.16          | 0.011      | 91.0             | 51.5       |
| 3        | Z-11                                              | 0.04  | 11.5 | 28.4          | 0.20       | 0.16          | 0.019      | 90.5             | 36.2       |
| 4        | {N-butylithiouronium chloride<br>NBC Oil<br>Z-11} | 0.007 | 11.5 | 25.6          | 0.20       | 0.16          | 0.016      | 91.0             | 44.0       |

This example shows the effect of NBC oil on recovery of molybdenum using a standard collector such as Z-11, the N-butylithiouronium chloride, and in combination with the referenced collectors. The addition of NBC oil with an isothiouronium chloride salt give an improvement of 15% in recovery over the results obtained with the standard reagent Z-11, of which 4.2% can be attributed directly to the NBC oil. The NBC oil is also compatible with combinations of the isothiouronium salt (a cationic) and the Z-11 (an anionic), giving 8% improvement over the results obtained by the standard Z-11.

#### EXAMPLE V

A domestic ore containing 1.49% copper and 6.75% Fe and no molybdenum sulfide was subjected to flotation

30 seconds (60 seconds if the collector was added to the flotation cell) with Dowfroth 250 and floated 5 minutes.

An additional flotation step, preceded by a collector addition and conditioning in the cell, was made for 3 65 minutes. The two rougher concentrates were combined and thickened. The thickened bulk concentrate was then reground in a ball mill for 5 minutes at approximately 45–50% solids. A minimum pH level of 11.9 was used in a cleaner flotation step. The reground pulps were diluted to about 20% solids in a 250-gram stainless steel Denver flotation cell (1200 r.p.m.) conditioned 15 seconds (1 minute, if additional collector was added to the cell) and floated 3 minutes, constituting the first cleaner flotation step. A second cleaner flotation product was collected for 70 2 minutes after another 15 second conditioning period.

The two cleaner products were combined as a bulk cleaner concentrate.

The bulk cleaner concentrates of copper and molybdenum obtained as described above were dewatered, and were subjected to a flotation process for the separation of molybdenum minerals from copper minerals, using various depressing agents for copper minerals in accordance with the following procedure.

The thickened copper-molybdenum bulk cleaner concentrate was subjected to the particular depressant system being tested by conditioning in a stainless steel beaker with an air-driven mixer. The conditioned pulps were then diluted in a 250-gram stainless steel Denver flotation cell (1200 r.p.m.), pH adjusted to 7.0-7.3 (except when the sodium sulfide depressant system was used, in which case the pH level was near 12.0), conditioned for 2 minutes and floated 4 minutes.

The rougher Mo concentrate thus obtained was then subjected to a second addition of the depressant system being tested. The conditioned pulp was then diluted to flotation density in a 250-gram stainless steel Denver flotation cell (1,000 r.p.m.), pH adjusted to 7.0-7.3, conditioned for 1 minute and floated for 3 minutes, the froth product from this step constituting the molybdenum concentrate. Test results are shown in Table VI.

TABLE VI

| Test No.     | Collector Used         | #/T           | pH            | Rougher Conc. |      | Agent used for depressing Cu Minerals                | Percent Distribution of Metals |      |                |      |
|--------------|------------------------|---------------|---------------|---------------|------|------------------------------------------------------|--------------------------------|------|----------------|------|
|              |                        |               |               | Cu            | Mo   |                                                      | Mo Concentrate                 |      | Cu Concentrate |      |
|              |                        |               |               |               |      |                                                      | Cu                             | Mo   | Cu             | Mo   |
| 485-299...   | Z-11 and Z-200.....    | {0.02<br>0.06 | {11.6<br>11.6 | 97.1          | 57.3 | "Nokes" reagent.....                                 | 4.7                            | 44.0 | 92.4           | 13.3 |
| 485-292...   | Z-11 and Z-200.....    | {0.02<br>0.06 | {11.6<br>11.6 | 95.5          | 56.4 | Sodium ferrocyanide and heat.....                    | 8.5                            | 46.8 | 87.0           | 9.6  |
| 485-307...   | Nitrogen distillate .. | 0.138         | 7.7           | 93.9          | 92.3 | Sodium sulfide.....                                  | 4.4                            | 82.5 | 89.5           | 9.8  |
| 485-256..... | do.....                | 0.115         | 7.9           | 93.4          | 90.6 | Sodium hydroxide and heat.....                       | 9.7                            | 77.4 | 83.7           | 13.2 |
| 485-295..... | do.....                | 0.138         | 7.7           | 91.2          | 88.9 | Potassium permanganate.....                          | 12.9                           | 78.4 | 78.3           | 10.5 |
| 485-302..... | do.....                | 0.138         | 7.6           | 92.1          | 92.6 | "Nokes" reagent.....                                 | 3.4                            | 52.4 | 89.7           | 40.2 |
| 485-294..... | do.....                | 0.138         | 7.9           | 93.2          | 92.0 | Sodium ferrocyanide, sodium hydroxide, and heat..... | 4.1                            | 53.7 | 89.1           | 38.3 |

Example VI shows the effect of using nitrogen distillate in testing as a bulk collector followed by depression tests using Nokes reagent and other depressants.

It will be noted that nitrogen distillate consistently floats more molybdenum minerals and that much better recovery of molybdenum is obtained in the resulting molybdenum concentrates in all of the depressant tests.

The laboratory examples noted above show that NBC oil is a multi-purpose reagent, both a bulk flotation collector by itself, a synergistic auxiliary reagent to the traditional sulfhydryl collectors (anionics) and isothiouronium salts (cationics), is a good copper collector with a tendency to depress pyrite on both copper and coppermolybdenum sulfide ores, is a good molybdenum collector on ores containing only molybdenum sulfide, and is also a froth modifier for the isothiouronium salts.

In the operations where both molybdenum and copper concentrates were collected through the use of the S-substituted isothiouronium salts and NBC oil, it was found that the use of sodium ferrocyanide as a depressant for the copper sulfide minerals was unusually effective, giving greater filterability of the molybdenum minerals and also of the copper minerals.

While in the foregoing specification we have set forth specific procedure in considerable detail for the purpose of illustrating embodiments of the invention, it will be understood that such details of procedure may be varied widely by those skilled in the art without departing from the spirit of our invention.

We claim:

1. In a process for the separation of molybdenum in metallic sulfide ores containing molybdenum and iron minerals, the steps of conditioning a water suspension of said ores in finely-divided condition with a mixture of heterocyclic nitrogen compounds extracted from the mineral gilsonite and having an average boiling point within the range of about 200° F. to 750° F., and separating molybdenum concentrate as froth product.

2. The process of claim 1 in which the heterocyclic nitrogen compounds are selected from the group consisting of nitrogen distillate and nitrogen bases concentrate oil.

3. The process of claim 2 in which the amount of the compound is about 0.005 to about 0.5 pound per ton of dry ore.

4. The process of claim 1 in which said metallic sulfide ores contain molybdenum, copper and iron, and molybdenum and copper concentrates are separated as froth product.

5. In a process for the separation of molybdenum and copper in metallic sulfide ores containing as metallic constituents molybdenum, copper and iron and in which said ores are finely ground and suspended in water containing lime, the steps of conditioning said ore with a mixture of

heterocyclic nitrogen compounds extracted from the mineral gilsonite and having an average boiling point within the range of about 200° F. to 750° F., and separating molybdenum and copper concentrate as froth product.

6. The process of claim 5 in which said conditioning with said heterocyclic nitrogen compound mixture is carried out in the presence of an auxiliary collector selected from the group consisting of alkyl and aryl dithiophosphates, dithiocarbonates, dithiocarbamates, thionocarbamates, thioureas, and xanthogen formates.

#### References Cited

#### UNITED STATES PATENTS

|    |           |         |                 |           |
|----|-----------|---------|-----------------|-----------|
| 55 | 1,281,018 | 10/1918 | Janney .....    | 209—166   |
|    | 1,350,364 | 8/1920  | Dosenbach ..... | 209—166   |
|    | 1,438,590 | 12/1922 | Forrest .....   | 209—166   |
|    | 1,490,736 | 4/1924  | Frederick ..... | 209—166   |
|    | 1,683,569 | 9/1928  | Klepko .....    | 209—166 X |
| 60 | 2,267,307 | 12/1941 | Ralston .....   | 209—166   |
|    | 2,287,274 | 6/1942  | Ralston .....   | 209—167   |
|    | 2,305,032 | 12/1942 | Read .....      | 209—166   |
|    | 2,336,868 | 12/1943 | Jayne .....     | 209—166   |
|    | 2,594,612 | 4/1952  | Bates .....     | 209—166   |
| 65 | 2,664,199 | 12/1953 | Barker .....    | 209—167   |

HARRY B. THORNTON, Primary Examiner.

R. HALPER, Assistant Examiner.